

## UNITED STATES PATENT OFFICE

2,570,566

TEXTILE TREATING SOLUTIONS AND  
COMPOSITIONS CONTAINING SAME

Frank Wesley Lane, Newport, and William Leonard Dills, Wilmington, Del., assignors to E. I. du Pont de Nemours & Company, Wilmington, Del., a corporation of Delaware

No Drawing. Application January 24, 1947,  
Serial No. 724,242

5 Claims. (Cl. 252—8.1)

1

This invention relates to new titanium-antimony compositions useful in treating cellulosic substances, especially textile materials, in order to impart valuable properties thereto. More particularly, it relates to the production of novel, relatively dilute, stable, monobasic acid solutions containing titanium and antimony useful for imparting flame-proof characteristics to textiles having a cellulosic base.

The cellulosic fabrics of commerce such as rayon and cotton goods are easily ignited in the presence of a flame, and when used in clothing of very light weight, or of heavier weight but having a pile finish, present appreciable fire hazards to the wearer. Pile fabrics are particularly disadvantageous in this respect because the cellulosic pile propagates a flame easily. As a consequence, clothing manufacture from these fabrics has been somewhat retarded in the trade despite the more attractive appearance which they present. This dangerous characteristic is so great that action by the American Association of Textile Chemists and Colorists has resulted in its providing a testing method for such fabrics to determine their flash or flame-resistance properties. In such test, a rectangle of the treated cloth, measuring 2" by 6", must be heated for 15 minutes at 105° C. and then cooled in a desiccator over calcium chloride. The resulting dried cloth must have a moisture content of less than .3%. The cooled cloth must then be removed while supported on a screen held at a 45° angle, and must be touched with a half-inch flame. To pass such test, even after laundering, pile goods must not show material flashing, while flat goods (tested in a vertical position) must not continue to burn after the flame is removed.

Various oxides have been added to or incorporated in fabrics to render them fire- or flame-proof. Processes employed for the purpose usually included the simultaneous use of a chlorinated resin or chlorinated paraffin to assist in obtaining the flame-proofing effect sought. Such methods, however, substantially change the nature of the goods under treatment by reason of the resin or paraffin addition, which disadvantageously alters the properties of the fabric and limits the extent of use of the flame-proofed material. Hence, fabrics so treated are not satisfactory for general clothing purposes. Furthermore, such treatment cannot be applied to pile goods, nor, following treatment, can the pile be easily raised on the flat goods. As a consequence, prior flame-proofed fabrics have not proved acceptable to clothing manufacturers because lack-

2

ing in consumer appeal, while untreated products, such as those made of cotton and rayon and particularly pile fabrics made from brushed viscose rayon, although possessing requisite consumer appeal, have met with resistance due to their substantial fire hazard risk.

Antimony solutions have also been used to treat textile materials, but these must be employed at such high concentrations of acidity that they become disadvantageous for use in treating certain textiles, particularly delicate cellulosic substances, due to the deleterious, injurious effects which they exert thereon. Relatively dilute solutions, on the other hand, are non-useful because unstable in nature and decompose to prematurely precipitate antimony oxide.

The disadvantages exhibited by prior textile treating solutions have greatly limited their utility in such field, and present a real need for a treating solution which is free from such disadvantages and is effectively useful for treating all forms of cellulosic textile materials, and more especially delicate cellulosic substances.

It is among the objects of this invention to overcome the above and other disadvantages characterizing prior cellulosic textile treating solutions, and to provide in particular a novel form of antimony-titanium monobasic acid solution, which, though in relatively dilute state, remains highly stable and is eminently satisfactory for treating or impregnating cellulosic substances in order to impart flame- and flash-resistant characteristics thereto. Further objects include the provision of a novel solution containing as an essential ingredient a dissolved complex titanium-antimony compound and methods for obtaining the same; the provision of a relatively dilute, stable halogen acid (especially chloride) solution of titanium and antimony which is resistant toward decomposition or hydrolysis in the presence of substantial amounts of aqueous media; the provision of a titanium-antimony solution which, when applied to a textile material, will provide a non-toxic, laundry-proof type of product and will be free from the injurious toxic and other effects attendant the use of antimony solutions upon textiles. A prime objective of the invention is to overcome the hazardous character toward fire which prior cellulosic fabrics employed as clothing have exhibited; while a further object is the production of cellulosic base fabrics which are flame-proof and remain substantially unchanged in appearance and feel after treatment. A still further object is to produce rayon and cotton goods having a high pile which will meet all

standards of the rigorous A. A. T. C. C. test above outlined. Other objects and advantages will be apparent from the ensuing description of our invention.

These and other objects are realized in this invention which embodies the discovery that certain monobasic acid solutions of titanium and antimony, and more especially halide (chloride) solutions thereof, are eminently useful, even under conditions of relatively high dilution, for treating cellulosic textile materials, and that the treated product results in a flame- and flash-proofed composition which will meet all requirements of the above A. A. T. C. C. test.

In practically applying the invention in accordance with one particular adaptation thereof, our stable, dilute antimony-titanium solution can be readily obtained by first combining at room temperatures commercial titanium tetrachloride with antimony oxide in the presence of water, and effecting the combination in such manner as will produce a dissolved complex titanium-antimony compound in which, preferably, the acid portion of the complex is supplied by hydrochloric acid and a ratio of 1 mol of HCl for each 2 mols of titanyl chloride and each mol of antimony chloride exists. Thus, titanium tetrachloride is first dissolved in cold water, following which the antimony oxide proportion is added to the resulting aqueous titanium solution, with such proportion of reagents being employed that the concentration of the oxides of titanium and antimony in the final solution will range, preferably, from 200 to 400 g./l. of the combined titanium and antimony oxides. To insure production of a stable solution free from any tendency to hydrolyze or precipitate antimony oxide, care must be taken to maintain in the solution a concentration of not less than 2.5 to 3 mols of chloride ions over and above those present in the  $\text{SbCl}_3$ . Such solutions exhibit excellent stability characteristics, even when relatively dilute and although they contain less chlorine than is necessary to form the normal chlorides of titanium and antimony, i. e., are basic. This stability is contrary to the characteristics of equivalent solutions in which titanium ions are not present. For commercial purposes and more economical shipping, solutions containing about 400 g./l. of the oxides of titanium and antimony are preferred. Prior to use, they can be readily adjusted to about 300 g./l. of the combined oxides.

As stated, the titanium-antimony solutions of the invention are useful in the treatment of cellulosic substances generally, especially those having hydroxy groups which are free to combine with titanium, and particularly materials, such as wood, cellulosic films, cloth, woven fabrics, paper, cellophane, etc., to impart flame- and flash-resistant properties thereto. Our novel solutions are outstandingly useful in the flame-proofing of cellulosic textile materials, including natural cellulose, such as cotton, artificial silks obtained from regenerated cellulose fibers from either the viscose, cellulose acetate, nitrocellulose or cuprammonium manufacturing processes, wherein use is resorted to of cellulose derivatives, such as cellulose esters (acetate, formate, butyrate, propionate, etc.) and ethers (notably ethyl cellulose, etc.); mixed cellulose esters or ethers (cellulose acetate propionate, cellulose nitrate acetate, methyl or ethyl cellulose acetate, etc.) and the like. In effecting textile treatment, the solution is preferably applied to the woven fabric, but obviously such treatment can be applied to

other forms of the textile, including knitted or netted fabrics, threads, yarns, fibers, etc. Advantageously, the textile, after treatment, though containing substantial amounts of antimony, is non-toxic and harmless in nature, a property in sharp contrast to that exhibited by compositions treated with antimony oxide alone, and which are known to be toxic and harmful in that they cause serious physiological effects after internal use or external application.

In treating the rayon, cotton, or like textile material with our solution to impart the desired flame-proofing characteristics thereto, it is first wetted by immersing it, for example, in a suitable bath containing the monobasic acid titanium-antimony solution and allowing it to remain therein for a period of time ample to allow the liquid to completely permeate the interstices and pores of such material. Alternatively, the impregnation can be effected by passing the material between suitable rollers suitably coated or wet with the impregnating solution. After such immersion and impregnation, it may be removed from the bath and passed through suitable nip or ringer rolls, or centrifuged, to remove excess treating solution and insure uniform treatment and impregnation throughout. The temperature of the immersing bath is usually maintained at about 25° C., but preferably ranges from 5° C. to 75° C., and should not be allowed to exceed about 90° C., so that no damage to the textile under treatment will take place. After impregnation, the product is passed into a suitable precipitating bath containing a precipitant capable of precipitating the titanium-antimony complex in insoluble form on the textile material. Among useful precipitants for the purpose are ammonium hydroxide and salts and alkali metal hydrates, as well as salts of the alkali metals. Specific examples of such precipitants include solutions of sodium carbonate, sodium hydroxide, potassium hydroxide, potassium carbonate, ammonium hydroxide, sodium silicate, sodium phosphate, phosphoric acid, benzoic acid, boric acid, etc. The precipitating bath is usually maintained at ordinary room temperature, but may be at higher or at lower temperatures and ranging from 5° C. to 100° C. Preferably, a dilute concentration of the precipitant is maintained in the bath, with solutions at from about 1% to 20% strengths being adequate for most purposes. The time treatment of the textile in the bath is variable and will depend upon its type and thickness.

Following precipitating bath treatment, the textile is next conventionally washed by passing it through a washing bath containing water or other suitable washing fluid, such as a soap solution, in which by-products of the reaction are removed and any loosely-held metal compounds, such as hydrated titanium and antimony oxides, which are easily removed by laundry treatments and are not firmly retained by the fabric, can be eliminated.

While our contemplated treatment may be applied to threads and yarns, it is usually applied to flat goods. When pile fabrics are being treated, the napping can be carried out either before or after the treatment as the flash-proof properties are not lost by subsequent brushing. Thus, the treatment provides an improved fabric on which our novel complex is firmly held and remains so held even after the drastic treatment given the goods during the napping operation and throughout subsequent launderings when in use.

To a clearer understanding of the invention, the following specific examples are given, which are merely illustrative and not to be taken as limiting the underlying principles or scope of the invention:

*Example I*

A titanium chloride solution was prepared by adding titanium tetrachloride to cold water to provide a concentration of 210 g./l.  $TiO_2$  and 382 g./l. HCl. Antimony trioxide was then dissolved in this solution to a concentration of 100 g./l., the final solution containing antimony oxide to the amount of 48% by weight of the  $TiO_2$  or 26% by weight of the HCl. The resulting product comprised a clear, yellow, homogeneous solution of a titanium-antimony complex, which solution, though dilute in nature, was highly stable and evidenced no tendency to hydrolyze or reprecipitate the antimony oxide. In contrast thereto, an equivalent antimony solution containing no titanium ions exhibited marked decomposition and hydrolysis, due to water presence.

*Example II*

A titanyl chloride solution containing 200 g./l.  $TiO_2$  and 365 g./l. HCl (approximately 1 mol of titanium to 4 mols of chlorine) was prepared by adding commercial titanium tetrachloride to ice-cold water. Sufficient antimony trioxide was then dissolved in this to give a concentration of 6.4 grams per liter. This represented an  $Sb_2O_3$  content of 3.2% by weight of  $TiO_2$  or 1.75% by weight of HCl. As in the instance of Example I, a clear, stable, yellow solution was obtained.

*Example III*

A titanyl chloride solution was made up having 1 mol of titanium to 3.4 mols of chlorine and a  $TiO_2$  content of 225 grams per liter with an HCl content of 348 grams per liter by adding commercial  $TiCl_4$  to ice-cold water. 168 grams per liter antimony trioxide were then dissolved in said solution, representing 75% by weight of the  $TiO_2$  and 48% by weight of the HCl. The resulting solution was diluted one-third with water, and still remained perfectly stable.

*Example IV*

A titanium chloride solution was prepared from anhydrous  $TiCl_4$  by adding the latter to cold water and diluting to 300 g./l.  $TiO_2$  and 497 g./l. HCl.  $Sb_2O_3$  was then dissolved in the resulting solution and sufficient water was added to give a solution containing 220 g./l.  $TiO_2$  and 165 g./l.  $Sb_2O_3$ . As in the instance of the above examples, a clear, stable, yellow solution was also obtained.

*Example V*

A titanium chloride solution was prepared from anhydrous titanium tetrachloride by adding the latter to water under conditions conducive to the evolution of gaseous HCl. The solution thus prepared analyzed 400 grams per liter  $TiO_2$  and 380 grams per liter HCl and contained slightly more than 2 mols of HCl per mol of titanium. This solution was mixed with an equal volume of antimony chloride solution analyzing 400 grams per liter  $Sb_2O_3$ . The mixed solution contained 200 grams  $TiO_2$  per liter and 200 grams per liter  $Sb_2O_3$ . Brushed viscose blanket material having  $\frac{1}{4}$  to  $\frac{1}{2}$ " pile was soaked in this solution for 5 minutes, wrung on a tight roll and after 15 minutes immersed in a saturated  $Na_2CO_3$  solution until neutral. The material was thoroughly scrubbed with soapy water and rinsed.

A sample of the treated fabric after air drying for 24 hours was heated for 15 minutes at 105° C. in a circulating oven and cooled to room temperature in a  $CaCl_2$  desiccator. The dried sample supported at a 45° angle, after the pile had been raised with a comb or brush, did not flash when a  $\frac{1}{2}$ " flame was impinged on its surface for 1 second. The treated sample contained 7.5%  $TiO_2$  and 7.5%  $Sb_2O_3$ .

10 After 20 complete washings in 0.5% Ivory soap flakes solution the treated sample was flame-proof when again tested as described above.

*Example VI*

15 Cotton sheeting material and flat viscose curtain material were dipped in the solution of Example IV and wrung on a tight roll. After 15 minutes the material was neutralized with saturated  $Na_2CO_3$  solution and washed to remove the loosely-held hydrous oxide precipitates. The air-dry samples heated 15 minutes at 105° C. and cooled in a  $CaCl_2$  desiccator, held in a vertical position and touched with a half-inch flame did not continue to burn after the flame was removed.

20 25 The treated cotton sheeting was tested after 15 washings and was still flame-proof by the A. A. T. C. C. test.

25 The flat viscose material washed 25 times still passed the flame test described, also demonstrating the laundry-proof character of the treatment.

30 Although described as applied to certain specific adaptations, the invention is not limited thereto. For instance, while hydrochloric acid solutions of antimony and titanium are particularly described and preferred for use, production is generally contemplated of stable, monobasic acid solutions containing both antimony and titanium as essential constituents. Thus, in lieu of the chloride, other monobasic acid solutions such as those of nitric acid, or of other halides, such as hydrogen bromide or hydrogen iodide, can be produced and utilized in the flameproofing of textiles, it being essential to these solutions, as in the case of the chloride, that they contain at least 2.5 atoms of the monobasic anion over and above that present in the antimony compound, with a concentration of from 2.5 to 5 atoms of said anion over and above said antimony compound comprising a preferred useful concentration.

35 Likewise, although solutions having concentrations of the combined titanium and antimony oxides ranging from 200-400 g./l. are preferred for use, solutions containing concentrations of such combined oxides ranging from 25 to 500 g./l. can also be employed. For commercial usage, solutions containing about 2 mols of titanium chloride for each mol of antimony chloride are most advantageously useful. On a weight basis, this is slightly less of

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255

provide sufficient treating agent to yield a treated fabric containing from about 8 to 16% combined metal oxides when applied to viscose goods. Obviously, the actual amount realized will depend on such things as the past history of the fabric, the length of time of contact of the solution with the fabric, the concentrations of solution used, the steps taken to remove excess solution from the fabric, and the like.

Again, while preferably the antimony and titanium complex of this invention is obtained by combining commercial titanium tetrachloride with antimony oxide,  $Sb_2O_3$ , in the presence of water, the invention is not limited to such reagents nor to such preferred method of obtaining the complex. Any soluble, monobasic acid salt of antimony and titanium, including their nitrates, chlorides, iodides, and bromides, can be employed in the mixing, as can the respective oxides of these metals. In utilizing titanium oxide, the  $TiO_2$  can be dissolved in hydrochloric acid followed by dilution with water of the resulting solution to the desired concentration. The titanium oxide combines in this instance with the  $HCl$  and forms titanyl chloride, the  $TiO^{++}$  ions of which appear to cause the desired effective stabilization. The quantity of titania used will depend upon the concentrations of the other components of the solution and the results desired, but in general the employment of about 1 mol of titanium to at least 2 mols of chlorine will usually provide satisfactory results. In addition to  $Sb_2O_3$ , other forms of antimony oxide can be used, including the tetra and penta oxides, as well as antimony oxychlorides. When antimony chloride is employed, it can be dissolved in water, provided the solution is acidified by the presence of free  $HCl$ , following which the antimony solution can be combined with the titanium solution.

While sodium carbonate comprises a preferred type of mildly-alkaline reagent or precipitant for the treated textile following its treatment with the titanium-antimony solution, other types of alkaline agents, such as sodium bicarbonate, ammonium carbonate, potassium carbonate, etc., may be employed. Similarly, washing of the neutralized fabric with a soap solution can be effected through the use of any type of detergent solution, such as ordinary laundry soaps adequate to remove loosely-adhering metal compounds and effect a desired cleaning of the fabric.

The stability exhibited by the dilute titanium-antimony solution of this invention appears to arise from the association of titanium and antimony ions with each other with resulting formation of a definite complex compound within the solution itself or in the fabric impregnated therewith. This is clearly demonstrable by means of light transmission measurements of a series of solutions consisting of (a) a molar antimony chloride solution containing 3 mols of  $HCl$ ; (b) a solution containing 2 mols of titanium chloride, designated as a  $TiOCl_2$  solution, containing 3 mols of  $HCl$  in excess of that required for the given formula of the titanium salt, but less chlorine than would be present in a solution resulting from the dissolution of  $TiCl_4$  in water; and (c) a combined solution containing 1 mol of  $SbCl_3$ , 2 mols of  $TiOCl_2$ , and, like the other two solutions, 3 mols of  $HCl$ . When curves are prepared on the basis of light transmission figures obtained by subjecting each solution to a conventional type quartz spectrophotometer, the

curve for the mixed solution occurs considerably to the right of the curves for the unmixed solutions, and substantially to the right of the calculated curve for such mixed solution. This deviation from the expected curve can only be explained by formation of a definite complex compound of titanium and antimony within the solution which prevents the antimony from behaving in its normal and expected manner.

As above outlined, this invention provides for the flash-proofing of high pile fabrics and particularly those made from cellulosic solutions, as by the viscose operation. When producing flash-proofed viscose fabrics, no changes are needed in the process up until the time the fabric is produced, as the treatment is well-suited for the production of flame-proofed articles from flat woven viscose textiles. It is of course possible to treat threads and fibers or even sheeted cellulosic structures such as transparent cellulosic films, but the invention is particularly applicable to fabrics intended for the production of high pile textiles, since this line of goods is in the greatest need for modification. The process is also useful in fire-proofing or flame-proofing cotton materials, flat viscose and other forms of regenerated cellulose, and cellulosic compounds such as acetate rayon. All such materials have a cellulosic base, and accordingly the invention is to be regarded as useful in the treatment of fabric material having this cellulosic base, regardless of whether it is a woven fabric or a sheet fabric.

While preferably and to obtain optimum benefits under the invention, the textile or fabric under treatment is immersed directly in a monobasic acid solution containing our titanium-antimony complex, alternatively such textile or fabric may be impregnated with a titanium chloride solution as the first step in the treating process, after which the impregnated cloth, without drying, is immersed in the antimony solution. Thereafter, the subsequent neutralization and washing treatments can be resorted to. While this method of treatment will afford flameproofing, the process is readily carried out and more effective results obtain when the cloth is subjected to treatment directly with the titanium-antimony complex solution. In this case, a single immersion of the goods or fabric in the acid-reacting solution is had and the after-treatment with alkali and scrubbing in soap solution is likewise simplified.

The mechanism of the treatment is not completely understood; but it is believed that the titanium is enabled to cling to the hydroxyl groups of the cellulose and become insolubilized thereby. The antimony may cling to the cellulose as well, or to the adhering titanium, but the point is not at present well understood or definitely ascertainable. One thing is certain, the flame-proofing of such fabrics is effectively realized, and there is provided a process for the manufacture of pile viscose fabrics, which may be used for the making of attractive garments having great consumer appeal. The herein-contemplated treatment gives fabrics which pass the exacting A. A. T. C. C. test, but a treatment by any one of the reagents alone will not give such result. It is essential that titanium be present and that preferably it comprises the major constituent, i. e., is at least 50% of the weight of the combined oxides used.

In addition to imparting flame-proofing characteristics to a textile material, our contemplated treatment also renders such material

mildew-resistant and increases drag and delustering characteristics.

We claim as our invention:

1. A flame-proofing solution for cellulosic substances comprising an aqueous solution of titanium and antimony in an inorganic monobasic acid, said solution containing at least 25 g./l. of the combined oxides of titanium and antimony, with the atom ratio of antimony to titanium not exceeding 2 and the weight ratio of titanium to antimony ranging up to 10. 10

2. A flame-proofing solution for cellulosic substances comprising an aqueous solution of titanium and antimony in hydrochloric acid, said solution containing at least 25 g./l. of the combined oxides of titanium and antimony, with the atom ratio of antimony to titanium not exceeding 2 and the weight ratio of titanium to antimony ranging up to 10. 15

3. A flame-proofing solution for cellulosic substances comprising an aqueous solution of titanium and antimony in hydrochloric acid, said solution containing from 25 to 500 g./l. of the combined oxides of titanium and antimony, with the atom ratio of antimony to titanium not exceeding 2 and the weight ratio of titanium to antimony ranging up to 10. 20

4. A flame-proofing solution for cellulosic textile material comprising an aqueous solution of titanium and antimony chlorides, said solution containing at least 25 g./l. of the combined oxides of titanium and antimony, and having an atom ratio of antimony to titanium not exceeding 2 and a weight ratio of titanium to antimony ranging up to 10. 25

5. A flameproofing solution for cellulosic tex-

tile material comprising an aqueous solution of titanium and antimony in hydrochloric acid, said solution containing from 200-400 g./l. of the combined oxides of titanium and antimony, with the atom ratio of antimony to titanium not exceeding 2 and the weight ratio of titanium to antimony ranging up to 10.

FRANK WESLEY LANE.  
WILLIAM LEONARD DILLS.

#### REFERENCES CITED

The following references are of record in the file of this patent:

#### UNITED STATES PATENTS

| Number    | Name            | Date           |
|-----------|-----------------|----------------|
| 723,088   | Warr            | Mar. 17, 1903  |
| 1,501,895 | Andrews et al.  | July 22, 1924  |
| 1,648,433 | White           | Nov. 8, 1927   |
| 1,996,089 | Thompson        | Apr. 2, 1935   |
| 2,036,862 | Dreyfus         | Apr. 7, 1936   |
| 2,095,028 | Craik           | Oct. 5, 1937   |
| 2,147,056 | Platt et al.    | Feb. 14, 1939  |
| 2,310,128 | Smith           | Feb. 2, 1943   |
| 2,395,922 | Timmons         | Mar. 5, 1946   |
| 2,416,447 | Laughlin et al. | Feb. 25, 1947  |
| 2,427,997 | White           | Sept. 25, 1947 |

#### FOREIGN PATENTS

| Number  | Country       | Date          |
|---------|---------------|---------------|
| 9,556   | Great Britain | of 1901       |
| 312,301 | Germany       | Jan. 14, 1923 |

#### OTHER REFERENCES

Emphraim, Inorganic Chemistry, 14th ed.  
(1943), Nordeman Pub. Co., N. Y., pages 331 and  
756.